

April 3, 1928.

1,664,589

N. L. CAMPBELL

FLOOR COVERING

Filed March 29, 1926



FIG 1



FIG 2

INVENTOR.  
Neil L. Campbell  
BY  
Allen Allen  
ATTORNEYS

## UNITED STATES PATENT OFFICE.

NEIL L. CAMPBELL, OF GLENDALE, OHIO, ASSIGNOR, BY MESNE ASSIGNMENTS, TO CARTHAGE MILLS INCORPORATED, OF CINCINNATI, OHIO, A CORPORATION OF OHIO.

## FLOOR COVERING.

Application filed March 29, 1926. Serial No. 98,144.

My invention relates to the production of floor coverings, such as rugs, runners and carpets, on an asphalt saturated felt base, or other similar inexpensive and strong base.

5 It is my object to provide a floor covering in which the top or wear surface has the characteristics of textile material, in that it is soft, and presents a coherent resilient body in which the fibrous material forms the

10 top.

I am aware that it has been suggested to make rugs, carpets and runners on a base of asphalt saturated felt, by attaching thereto a piece of carpet material, or other woven 15 or otherwise formed fabric, or a stout all-rag felt, on which is a previously printed design, or which may be subsequently printed.

I am also aware that it has been suggested to make a floor covering in which a piece of textile fabric is completely embedded in an asphaltic or other bituminous or resinous coating which serves to secure 20 it to a saturated felt base, so as to form a surface which bears a fabric imprint, on which a design is painted.

According to my process I proceed in the formation of a wear surface on the usual asphalt saturated felt base, by first imprinting upon the felt base, a substance which 30 through long practice has been developed to have very tight adherence thereto, and a very hard, but resilient quality over a long period of time: to wit, floor coating paint.

35 By floor coating paint, I refer to that nature of paint which has for many years been applied to asphalt base and linoleum bases, upon the dried surface of which is printed a pattern or design by means of suitable printing apparatus or by hand. The designs are also printed with paint of the same or similar nature. This paint is characterized by the inclusion of polymerizing substances such as China-wood oil which 40 upon an oven treatment gives the paint a very hard, but resilient characteristic, providing a long lasting surface highly inert to chemical action and heat.

45 I apply to a piece of asphalt saturated felt or other floor covering a surface of coating paint which is then brought to the

thickened condition by partial drying or the paint is given an initial thick body and tackiness arising from cutting down the linseed oil content, and using quick dryers and 50 a large proportion of pigments and other substances known to the painters art to give a thick body. While the paint is tacky, a piece of such fabric as may be desired, is rolled down onto the sticky paint surface. 55

Due to the skill acquired in the trade over many years in getting a full bodied, tightly adherent and uniform coat of coating paint on a piece of felt or linoleum floor covering, it is a matter of selection between various 60 methods known to composition flooring makers, to provide a body of paint onto which the fabric may be pressed, which paint is in the condition described.

Thus the paint can readily be given 65 enough body, either by partial drying or by using a thick and quick drying paint to begin with and at once applying the fabric, so that it will not penetrate through to the surface of the fabric, but will penetrate far 70 enough to incorporate the lower surface thereof into the paint, and this is what is done by me.

75 After the fabric has been applied and the product has been baked and tempered in the usual oven, the fabric will be found to be permanently and tightly bound to the base, by a resilient, hard, long wearing body, which has a very tight and complete bond, both with the felt base and the fabric. 80

As a fabric I prefer to employ one which has a wooly quality, because its thickness will enhance the softness of the final product. Also a closely woven or a full napped 85 fabric, will find more places of contact with the paint, and be more tightly built into the product.

In the drawing:

Figure 1 is a diagram showing the process.

Figure 2 is a perspective of the final 90 product.

I can use the machines used in making painted, asphalt saturated felt floor coverings, and in a typical example proceed with a piece of saturated felt 1, such as is used at 95 present in printing, and first imprint thereon by a roll, or preferably by several blocks

having the printing surfaces lined to completely cover the felt with imprint, a ground coat 2 of a thick, and almost gummy floor covering coating paint. This I find to be better than to print a heavy ground coat and let it partially dry.

In my typical process, I then pass the fabric 3 from a roll, onto the painted surface, and pass both the saturated felt and the fabric adhering thereto, beneath one or more rolls 4, which apply pressure and force the fabric down on the painted surface.

I then move the united body along a table to a printing mechanism, such as is used in printing flooring, and may use either paints or dyes in imprinting the fabric with whatever pattern is desired. At 5 I indicate a printing block, of which it is customary to use a series.

20 An alternative process for applying the coating paint, which I have used with success is to pass the base sheet of material, through a bath of the paint, and doctor it, and then apply the wear surface fabric as a 25 previously printed or dyed body, on one side of the base sheet, and a piece of burlap on the other, to serve as a back.

I place particular importance on the fact that the processing to make floor coverings 30 of my invention demands the learning of no new procedure in practicing it, as might be the case with glue or other agents. Floor coating paints in the floor covering industry are well known. They have qualities of 35 inertness to heat and chemicals, resilience, long wearing under the strains attendant upon floor coverings, and the application thereof to sheets of suitable base material are well known. Most important, also is 40 their quality of tempering in an oven so as to become very tough.

The nature of the base sheet is not necessarily particularized. I have mentioned asphalt saturated felt because it has well 45 known wearing qualities and is not pervious to moisture, and thus will lie flat when exposed for use. Thus unsaturated or partly saturated felts, roofing felts and the like can be used, or other inexpensive sheets of fabric 50 or felted composition.

I may or may not print the fabric after it is applied, and one of the advantages of the use of coating paint, lies in the fact that it is simple to give it a thick enough body so 55 that it will embed the back of a piece of textile fabric, but not come through to the wear surface thereof, thereby avoiding the necessity of a subsequent printing.

Finally, while it might appear that rubber 60 compositions, asphalts, glues and the like, would serve instead of a ground coat of paint, for my purpose, as an adhesive body, still this is not the case, since a rug carpet or runner becomes soiled and has to be 65 cleaned, and the usual cleansing agents will

soften asphalt, or rubber cement, and often other types of cementing coatings, and the cementing agent will then run through and stain or stiffen the wear surface. Also, if asphalt saturated felt is used as a base, it is necessary to have a protection over its surface to prevent cleansing agents from bringing the saturant to the wear surface. Coating paint has a known quality of imparting such a protection, and furthermore, when it is oven tempered it has the quality of long resistance to wear, and is tough, impervious to most of chemicals, which would not destroy the entire product, and stays permanently in its original condition.

To continue with the process, the material, when the fabric has been applied to one or both sides and after it has been passed between rolls to embed the fabric, is then passed into an oven, where heat is applied 80 to harden and temper the coating.

The final product may be cut into rugs 6, if the wear surface fabric is so printed as to permit this, or carpet strips or runners may be formed therefrom.

I make no specification of any additional treatments such as binding, stitching or the like, as these may or may not be used, without departing from my invention.

Having thus described my invention, what I claim as new and desire to secure by Letters Patent, is:—

1. A floor covering comprising a sheet of material as a base, a coat of paint thereon having the quality of being hard when dry, and a textile material embedded into the paint, with none of said paint penetrating to the upper surface thereof.

2. A floor covering comprising a sheet of material as a base, a coat of floor covering coating paint thereon, and a textile material embedded into the paint, with none of the said paint penetrating to the upper surface thereof.

3. A floor covering comprising a base of asphalt saturated felt, a coat of floor covering coating paint, as in a ground coat on said felt, and a textile fabric embedded into the paint with none of said paint penetrating to the upper surface thereof.

4. A floor covering comprising a sheet of material as a base, a coat of paint which has been oven treated and rendered hard, and a textile material embedded into the paint, with none of said paint penetrating to the upper surface thereof, and a design imprinted upon the said textile fabric.

5. A floor covering comprising a sheet of material as a base, a coat of oven treated floor covering paint thereon, and a textile material embedded into the paint, with none of the said paint penetrating to the upper surface thereof, and a design imprinted upon the said textile fabric.

6. A floor covering comprising a base of

asphalt saturated felt, a coat of oven treated floor covering paint, as in a ground coat on said felt, and a textile fabric embedded into the paint with none of said paint penetrating to the upper surface thereof, and a design imprinted upon the said textile fabric.

7. A process of forming floor covering which consists in ground coating a piece of flexible base material with paint, which is or becomes thick and tenacious and then applying thereto a strip of textile material,

rolling said material into the paint, and finally oven treating the product.

8. A process of forming floor covering which consists in ground coating a piece of asphalt saturated felt with paint, which is or becomes thick and tenacious and then applying thereto a strip of textile material, rolling said material into the paint, and finally tempering the product in an oven.

NEIL L. CAMPBELL.